

# United States Patent

[19]

Jasper et al.

[11] 3,905,780

[45] Sept. 16, 1975

[54] **OXIDATION-RESISTANT LOW ALLOY STEEL WITH AL COATING**

[75] Inventors: **Joseph C. Jasper; Marvin B. Pierson**, both of Middletown, Ohio

[73] Assignee: **Armco Steel Corporation**, Middletown, Ohio

[22] Filed: **June 25, 1973**

[21] Appl. No.: **373,278**

[52] U.S. Cl..... **29/196.2; 75/124; 117/114 C**

[51] Int. Cl..... **B32b 15/00**

[58] Field of Search..... **29/196.2; 75/124; 117/114 C; 148/37, 31.5**

[56] **References Cited**

UNITED STATES PATENTS

|           |         |               |          |
|-----------|---------|---------------|----------|
| 2,825,669 | 6/1955  | Herzog.....   | 75/124 X |
| 2,839,826 | 6/1958  | Farrell ..... | 29/196.2 |
| 2,937,435 | 5/1960  | Brenner ..... | 29/196.2 |
| 2,965,963 | 12/1960 | Batz.....     | 29/196.2 |

|           |         |                |          |
|-----------|---------|----------------|----------|
| 3,059,326 | 10/1962 | Jominy.....    | 29/196.2 |
| 3,378,360 | 4/1968  | McFarland..... | 29/196.2 |
| 3,698,964 | 10/1972 | Caule.....     | 75/124 X |

Primary Examiner—L. Dewayne Rutledge

Assistant Examiner—Arthur J. Steiner

Attorney, Agent, or Firm—Melville, Strasser, Foster & Hoffman

[57] **ABSTRACT**

A low alloy steel for use as a substrate for aluminum or aluminum alloy coatings, the steel containing from 0.01 percent to 0.13 percent carbon, from 0.5 percent to 3 percent chromium, from 0.8 percent to 3 percent aluminum, from 0.4 percent to 1.5 percent silicon, from 0.1 percent to 0.6 percent manganese, from 0.1 percent to 1 percent titanium and remainder substantially iron. The steel has good oxidation resistance at elevated temperature, good weldability and formability, thereby enhancing its utility for fabrication into a variety of wrought coated products.

**5 Claims, No Drawings**

# OXIDATION-RESISTANT LOW ALLOY STEEL WITH AL COATING

## BACKGROUND OF THE INVENTION

### 1. Field of the Invention

This invention relates to a chromium-aluminum-silicon-titanium steel of low alloy content for use as a substrate for aluminum or aluminum alloy coatings, and wrought coated products thereof having good resistance to oxidation at elevated temperatures up to about 1,700°F, and resistance against attack by hydrocarbon combustion products at elevated temperature, together with high strength.

### 2. Description of the Prior Art

Increasingly stringent requirements for antipollution controls on motor vehicles has created a need for relatively low cost alloys which will be oxidation resistant at elevated temperatures, for use in automotive exhaust systems, such as catalytic converters, mufflers, and like articles.

Aluminum coated carbon steel has proved to be not completely satisfactory for some high temperature applications. The automotive industry has substituted stainless steels such as Armco 409 (containing 0.05 percent carbon, 11 percent chromium, traces of aluminum, residual nickel, 0.5 percent titanium and remainder iron) and other stainless steels containing 11 percent or more chromium. The cost of such steel is high, thus making it undesirable for proposed use in automotive exhaust systems, such as catalytic converters, and the like. Moreover, although this stainless steel has fair oxidation resistance at elevated temperature, and good formability, it does not adequately withstand attack by molten salts and hydrocarbon combustion products at elevated temperature. The provision of an aluminum coating on such a steel has been found to result in a product having the desired properties, but this solution obviously adds even greater cost.

U.S. Pat. No. 3,698,964, issued Oct. 17, 1972, to E. J. Caule et al, discloses an iron base alloy with good oxidation resistance at temperatures of about 700° to 800°C (about 1,300° to 1,475°F). The alloy of this patent contains up to 2 percent carbon, 1 percent to 5 percent chromium, 1 percent to 4 percent aluminum, and/or 1 percent to 4 percent silicon, up to 1.5 percent manganese, up to 2 percent copper, up to 0.20 percent total of nickel, molybdenum, vanadium and other alloying elements. Preferably, a combination of 2 percent chromium and 3 percent aluminum, or 3 percent chromium and 2 percent silicon, are used, with manganese preferably up to 0.2 percent, copper not more than 0.5 percent, carbon not more than 1 percent and most preferably from 0.01 percent to 0.25 percent.

The high carbon content of the steel of the Caule et al patent results in a brittle structure having very limited cold workability, poor welding characteristics, and poor mechanical properties generally. The optional presence of molybdenum and vanadium adversely affects oxidation scale resistance, as well as adding to the cost. The harmful effect of molybdenum on oxidation resistance is reported in "Stainless And Heat Resisting Steels," by Colombier and Hochmann, p. 330, St. Martin's Press, New York, N.Y. (1968). Moreover, copper, nickel, and other austenite stabilizers in amounts greater than typical residual contents of about 0.2 percent each are undesirable since it can cause a phase change, with a consequent change in volume, on heat-

ing and cooling. This volume change results in spalling after cyclic heating and cooling.

U.S. Pat. No. 2,835,669, issued Mar. 4, 1958, to E. M. Herzog, discloses a steel, and a heat treatment therefor wherein a micro-structure is produced having resistance to stress-corrosion cracking in wet hydrogen sulfide atmospheres. The steel of this patent contains from 0.08 percent to 0.20 percent carbon, from 0.60 percent to 5.0 percent chromium, from 0.15 percent to 1.20 percent aluminum, from 0.30 percent to 1.20 percent manganese, from 0.10 percent to 0.50 percent silicon, up to 0.50 percent molybdenum, up to 1.0 percent vanadium, up to 1.0 percent titanium and remainder iron. A heat treatment at 740° to 780°C, a second heat treatment at about 970° to 1080°C followed by a waterquench and a tempering treatment at about 625° to 670°C, are stated to result in the desired micro-structure and an ultimate tensile strength of at least 95 ksi. Oxidation resistance at elevated temperature is not contemplated in this patent, and the composition would not inherently produce a steel having this property. Moreover, the presence of molybdenum and vanadium is deleterious for reasons set forth above. Other patents disclosing low alloy steels containing chromium, aluminum, and/or silicon in varying amounts include U.S. Pat. Nos. 3,431,101; 2,835,570; and 2,770,563.

None of the above patents discloses a low alloy steel having a completely ferritic structure within the contemplated operating temperature range, and exhibiting in combination good oxidation resistance at elevated temperature, good resistance against attack by hydrocarbon combustion products, good weldability and formability and relatively high strength. Hence, there still exists a great need for a low-cost alloy having the above combination of properties for fabrication into coated, welded and wrought products such as space heaters, automotive exhaust systems, e.g., catalytic converters and mufflers, and the like.

## SUMMARY

The present invention provides a low alloy steel containing chromium, aluminum, silicon and titanium (preferably with a total alloy content of less than about 5 percent) which provides in sheet form a substrate for aluminum or aluminum alloy coatings, the coated sheet being readily formable into wrought articles having good oxidation resistance at elevated temperature, good resistance against attack by hydrocarbon combustion products at elevated temperature, and relatively high retained strength at elevated temperature. In its broad composition ranges, the steel of the invention consists essentially of from about 0.01 percent to about 0.13 percent carbon, from about 0.5 percent to about 3 percent chromium, from about 0.8 percent to about 3 percent aluminum, from about 0.4 percent to about 1.5 percent silicon, from about 0.1 percent to about 0.6 percent manganese, from about 0.1 percent to about 1 percent titanium, and remainder iron except for incidental impurities. Molybdenum and vanadium are restricted to a maximum of about 0.05 percent each, and copper, nickel and other austenite stabilizers to less than about 0.2 percent each.

The carbon, chromium, aluminum, silicon and titanium percentage ranges are critical and departure therefrom results in loss of one or more of the above properties. Control of the critically low molybdenum,

vanadium, copper, nickel and other austenite stabilizer contents is also essential.

Carbon is essential in an amount of at least about 0.01 percent in order to provide the necessary strength in the steel. More than about 0.13 percent carbon cannot be tolerated because of its adverse effect upon the weldability, formability and general mechanical properties of the steel, and because it is a strong austenite former.

At least 0.5 percent chromium in combination with at least about 0.8 percent aluminum and about 0.4 percent silicon is necessary in order to provide good oxidation resistance. A maximum of 3 percent chromium should be observed in order to minimize cost and avoid processing difficulties.

At least about 0.8 percent aluminum is necessary not only for oxidation resistance at elevated temperature but also to provide adequate tensile strength. More than 3 percent aluminum results in a loss of formability and workability.

At least about 0.4 percent silicon is essential since it co-operates with the chromium and aluminum to impart oxidation resistance. However, a maximum of about 1.5 percent silicon should be observed since amounts in excess thereof also result in loss of formability and workability.

Titanium is essential in an amount of at least about 0.1 percent in order to impart good weldability to the steel. Moreover, excess titanium over that needed to stabilize carbon has been found to improve the oxidation resistance at elevated temperature. This excess can be slight in view of the high cost of titanium and of the relatively low residual sulfur, nitrogen and oxygen contents of the steel of the invention. Preferably the titanium content is 8 times the carbon content, and a maximum of about 1 percent titanium should thus be observed at the carbon levels contemplated herein. Since it is known that columbium and/or zirconium generally function in an equivalent manner in stainless steels, it is considered within the scope of the invention to substitute columbium and/or zirconium in whole or in part for titanium. Such substitution would be on a stoichiometric basis, with a minimum weight ratio of columbium or zirconium to carbon of 8:1, preferably at least about 10:1. Columbium and/or zirconium would thus range from about 0.10 percent to about 1.5 percent if substituted for titanium.

Impurities at residual levels normal for ferritic stainless steels can be tolerated in the steel of the invention. More specifically, a maximum of about 0.03 percent sulfur and a maximum of about 0.04 percent phosphorus do not adversely affect the properties of the steel. Molybdenum and vanadium are undesirable in the steel of the invention as explained above, and are maintained at the minimum practicable levels. Copper and nickel are maintained at a maximum of less than 0.2 percent each for reasons set forth above.

#### DESCRIPTION OF THE PREFERRED EMBODIMENTS

While the desirable novel combination of properties is achieved in a steel having the broad composition ranges hereinabove set forth, optimum properties are obtained in a steel having the following preferred analysis by weight percent:

|           |                           |
|-----------|---------------------------|
| Carbon    | about 0.04 to about 0.06% |
| Chromium  | about 1.7 to about 2.1 %  |
| Aluminum  | about 1.7 to about 2.0 %  |
| Silicon   | about 0.6 to about 0.9 %  |
| Manganese | about 0.2 to about 0.4 %  |
| Titanium  | about 0.1 to about 0.6 %  |

the titanium being about 8 times the carbon content and remainder iron except for incidental impurities.

In order to investigate the effect of the relative proportions of chromium, aluminum, silicon and titanium on the properties of the steel, a series of experimental heats was prepared and tested. For purposes of comparison, tests were also conducted on plain carbon steel coated with aluminum and aluminum alloys containing up to 10 percent silicon, and on Armco Type 409 stainless steel. The compositions of the experimental heats are set forth in Table I below.

TABLE I

| Sample Code | C     | Cr  | Al   | Si   | Mn   | Ti   |
|-------------|-------|-----|------|------|------|------|
| 15          | 0.048 | 1.0 | <0.1 | 0.2  | 0.3  | 0.4  |
| 41*         | 0.033 | .5  | 1.7  | 0.8  | 0.4  | 0.4  |
| 42*         | 0.033 | 1.0 | 1.7  | 0.7  | 0.4  | 0.4  |
| 43*         | 0.034 | 1.5 | 1.7  | 0.7  | 0.4  | 0.4  |
| 61*         | 0.037 | 1.0 | 1.0  | 0.7  | 0.4  | 0.3  |
| 62*         | 0.038 | 1.7 | .9   | 0.8  | 0.4  | 0.3  |
| 85          | 0.054 | 2.5 | 1.9  | 0.47 | 0.21 | 0    |
| 86*         | 0.073 | 2.0 | 1.92 | 0.81 | 0.32 | 0.48 |

\*Steels of the invention - also containing 0.1% Cu, 0.04% Mo, and 0.03% V.

The above materials were hot rolled from 2,100° F (1,149° C) from 1 inch by 3 inch ingots to 0.1 inch thickness. Samples were annealed at 1,700° F (927° C) for 10 minutes, descaled and cold rolled to 0.05 inch thickness. It should be recognized that annealing the hot rolled material is optional. Tensile strengths were determined on the cold rolled samples at this stage while the remainder of the cold rolled strip was annealed at 1,600° F (871° C) for 6 minutes and pickled. This material was tested for the remaining mechanical properties reported below in Table II.

A consideration of the mechanical properties reported in Table II indicates that the steels of the invention have ultimate tensile strengths equivalent to those of comparable prior art alloys but have improved elongation. This is believed to result from the relatively low carbon contents (ranging from about 0.03 percent to about 0.07 percent). The yield strength and tensile strengths of the alloys containing about 1 percent aluminum were about 5 ksi and 4 ksi, respectively, less than those containing 2 percent aluminum. Of greater significance is the comparison with the 1 percent chromium alloy (Sample Code 15) also having low aluminum and silicon contents. It will be noted that the yield strength of the 1 percent chromium alloy was about 12 ksi lower and the tensile strength about 8 ksi lower than the steels of the invention containing from about 1.7 percent to about 2 percent aluminum with chromium ranging from 0.5 percent to 2 percent. At the same time the elongation values of these steels of the invention were about equivalent to that of Sample Code 15. For an optimum combination of mechanical properties, it is thus apparent that the carbon content should not exceed about 0.06 percent, that aluminum should range from about 1.7 to about 2 percent in combination with at least about 1.7 percent chromium and at least about 0.6 percent silicon.

TABLE II

| Sample Code | 0.2% YS (ksi) | UTS (ksi) | % Elong. in 2" | Hardness (Rockwell B) | Olsen Cup Test Height-Inches |
|-------------|---------------|-----------|----------------|-----------------------|------------------------------|
| 15          | 23.65         | 53.95     | 35.5           | 57.0                  | .390, .430                   |
| 41*         | 36.40         | 61.85     | 36.0           | 73.0                  | .400, .410                   |
| 42*         | 35.65         | 62.15     | 34.0           | 73.0                  | .410, .405                   |
| 43*         | 35.80         | 62.55     | 35.5           | 73.0                  | .400, .400                   |
| 61*         | 29.95         | 58.25     | 37.0           | 68.0                  | .380, .400                   |
| 62*         | 30.45         | 58.60     | 34.5           | 68.5                  | .395, .440                   |
| 85          | 39.70         | 61.25     | 20.5           | 73.0                  | .390, —                      |
| 86*         | 37.15         | 61.10     | 26.0           | 73.0                  | .408, —                      |

\*Steels of the present invention

Samples of the steels of Table I in the cold rolled, annealed and pickled condition were surface ground, and a full penetration autogenous GTA weld was run down the longitudinal axis of the strip of each sample. 180° bend and Olsen cup test specimens were cut from the samples and tested with both root and face side in tension. These tests are reported in Table III.

From the data in Table III it is evident that optimum as-welded ductility is exhibited with about 1 percent aluminum and chromium in excess of 1 percent. At the 2 percent aluminum level better results apparently are obtained with chromium at about 2 percent.

The necessity for the presence of titanium for good weld properties is demonstrated by Sample Code 85, wherein a poor Olsen cup value was obtained. In addition, Sample Codes 85 and 86 were subjected to a further bend test across the weld (not reported in Table III), and it was found that Sample Code 85 cracked at 90° across the weld, whereas Sample Code 86 passed 180° flat across the weld.

For the coated specimens, a pure aluminum coating was applied by hot-dipping using a Lundin flux, details of which are disclosed in U.S. Pat. Nos. 2,686,354 and 2,686,355. Coating weight was about  $\frac{1}{2}$  ounce per square foot of sheet (total coating weight on both surfaces). For purposes of comparison, oxidation tests were also run on plain carbon steel coated with pure aluminum and with aluminum alloy containing up to 10 percent silicon, uncoated Armco Type 409 stainless steel, and an uncoated commercial alloy containing 5 percent chromium, 0.5 percent molybdenum, 0.06 percent carbon, 0.35 percent silicon, 0.4 percent manganese, residual aluminum and nickel, and balance substantially iron. The initial tests comprised 100 hours in still air at 1600° F, and 1700° F, respectively. These tests are reported in Table IV below.

Since still air tests are not necessarily definitive, further specimens of coated and uncoated materials were subjected to cyclic testing, using a cycle of 25 minutes

TABLE III

| Sample Code | As-Welded Properties            |                         |                               |                         |                              |                 |                 |                 |
|-------------|---------------------------------|-------------------------|-------------------------------|-------------------------|------------------------------|-----------------|-----------------|-----------------|
|             | 180° Bend Test Parallel to Weld |                         |                               |                         | Olsen Cup Test Height-Inches |                 |                 |                 |
|             | Root in Tension<br>.12" diam.   | Face in Tension<br>Flat | Root in Tension<br>.12" diam. | Face in Tension<br>Flat | Root in Tension              | Face in Tension | Root in Tension | Face in Tension |
| 15          | P.F                             | P.F                     | P.P                           | P.P                     | .310, .290                   | .340, .360      | —               | —               |
| 41*         | P.P                             | P.P                     | F.F                           | F.F                     | .300, .225                   | .300, .350      | .305, .340      | —               |
| 42*         | P.P                             | P.P                     | P.P                           | F.F                     | .300, .225                   | .400, .370      | .350, .350      | —               |
| 43*         | P.P                             | P.P                     | P.P                           | P.F                     | .370, .370                   | .350, .390      | —               | —               |
| 61*         | P.P                             | P.P                     | P.P                           | P.P                     | .405, .390                   | .380, .400      | —               | —               |
| 62*         | P.P                             | P.P                     | P.P                           | P.P                     | .380, .315                   | .370, .310      | —               | —               |
| 85          | —                               | P.P                     | —                             | P.P                     | .065                         | —               | —               | —               |
| 86*         | —                               | P.P                     | —                             | P.P                     | .360                         | —               | —               | —               |

P = Pass

F = Fail

\*Steels of the Invention

Duplicate tests in each condition

Oxidation resistance tests were conducted on the samples of Table I in the cold rolled, annealed and pickled condition, both on coated and uncoated speci-

mens. For the coated specimens, a pure aluminum coating was applied by hot-dipping using a Lundin flux, details of which are disclosed in U.S. Pat. Nos. 2,686,354 and 2,686,355. Coating weight was about  $\frac{1}{2}$  ounce per square foot of sheet (total coating weight on both surfaces). For purposes of comparison, oxidation tests were also run on plain carbon steel coated with pure aluminum and with aluminum alloy containing up to 10 percent silicon, uncoated Armco Type 409 stainless steel, and an uncoated commercial alloy containing 5 percent chromium, 0.5 percent molybdenum, 0.06 percent carbon, 0.35 percent silicon, 0.4 percent manganese, residual aluminum and nickel, and balance substantially iron. The initial tests comprised 100 hours in still air at 1600° F, and 1700° F, respectively. These tests are reported in Table IV below.

TABLE IV

| Sample Code                   | Oxidation Tests<br>100 Hours Still Air           |                                                  |
|-------------------------------|--------------------------------------------------|--------------------------------------------------|
|                               | 1600° F<br>Weight Increase<br>mg/in <sup>2</sup> | 1700° F<br>Weight Increase<br>mg/in <sup>2</sup> |
| Al-coated carbon steel        | 22.0                                             | 48.0                                             |
| Al-10% Si-coated carbon steel | 26.5                                             | 105.0                                            |
| Type 409 stainless uncoated   | 354.0                                            | 357.0                                            |
| 5% Cr-0.5% Mo uncoated        | 11.5 (loss from scaling)                         | 408.0                                            |
| 15 uncoated                   | 716.0                                            | 2070.0                                           |

TABLE IV—Continued

| Sample Code  | Oxidation Tests<br>100 Hours Still Air           |                                                  |
|--------------|--------------------------------------------------|--------------------------------------------------|
|              | 1600° F<br>Weight Increase<br>mg/in <sup>2</sup> | 1700° F<br>Weight Increase<br>mg/in <sup>2</sup> |
| 41 uncoated  | 7.6                                              | 14.1                                             |
| 42 uncoated  | 6.7                                              | 11.3                                             |
| 43 uncoated  | 4.1                                              | 7.8                                              |
| 61 uncoated  | 12.8                                             | 14.2                                             |
| 62 uncoated  | 6.3                                              | 19.3                                             |
| 85 uncoated  | 18.1                                             | 25.0                                             |
| 86 uncoated  | 2.1                                              | 3.9                                              |
| 15 Al coated | 15.8                                             | 30.2                                             |
| 41 Al coated | 12.5                                             | 11.1                                             |
| 42 Al coated | 16.2                                             | 10.0                                             |
| 43 Al coated | 13.6                                             | 10.0                                             |
| 61 Al coated | 14.8                                             | 13.6                                             |
| 62 Al coated | 16.6                                             | 9.8                                              |
| 86 Al coated | 6.1                                              | 6.2                                              |

TABLE V

| Sample Code   | Oxidation Tests<br>Cyclic 25/5 |                                       |
|---------------|--------------------------------|---------------------------------------|
|               | Conditions                     | Weight Increase<br>mg/in <sup>2</sup> |
| Type          |                                |                                       |
| 409 stainless | 135 cycles — 1500°F            | 118                                   |
| 15 uncoated   | 135 cycles — 1500°F            | 666                                   |
| 41 uncoated   | 135 cycles — 1500°F            | 315                                   |
| 42 uncoated   | 135 cycles — 1500°F            | 270                                   |
| 43 uncoated   | 135 cycles — 1500°F            | 250                                   |
| 61 uncoated   | 135 cycles — 1500°F            | 382                                   |
| 62 uncoated   | 135 cycles — 1500°F            | 376                                   |
| 85 uncoated   | 132 cycles — 1500°F            | 198                                   |
| 86 uncoated   | 132 cycles — 1500°F            | 117                                   |
| 15 Al coated  | 135 cycles — 1500°F            | 37.2                                  |
| 41 Al coated  | 135 cycles — 1500°F            | 17.4                                  |
| 42 Al coated  | 135 cycles — 1500°F            | 15.0                                  |
| 43 Al coated  | 135 cycles — 1500°F            | 12.3                                  |
| 61 Al coated  | 135 cycles — 1500°F            | 14.3                                  |
| 62 Al coated  | 135 cycles — 1500°F            | 18.2                                  |
| 86 Al coated  | 130 cycles — 1600°F            | 10.2                                  |

The oxidation tests indicate that all the steels of the present invention exhibited good scaling resistance both in still air and cyclic tests without coatings. With aluminum coatings, the steels of the invention are superior to Armco Type 409 in uncoated condition. It should further be noted that the still air tests on aluminum and aluminum alloy coated plain carbon steel base metal or substrate showed this material to be completely unacceptable for oxidation resistance at elevated temperatures of the order of 1,500° — 1,700° F, because of blistering and warpage.

Optimum oxidation resistance is achieved in a steel of the invention containing about 2 percent chromium, about 2 percent aluminum, about 1 percent silicon and about 0.5 percent titanium (with titanium about 8 times the carbon content). Sample Code 86, having this approximate analysis, was superior to other samples in the coated condition despite the fact that it was subjected to cyclic test temperatures 100°F degrees higher than any of the other materials tested. In the uncoated condition it was at least equivalent to other uncoated samples.

The embodiments of the invention in which an exclusive property or privilege is claimed are defined as follows:

1. An article having good oxidation resistance at elevated temperature, good resistance against attack by hydrocarbon combustion products at elevated temper-

ature, good formability, and high strength, said article consisting of an outer layer applied by hot dip coating chosen from the class consisting of aluminum, and aluminum alloys, and a ferritic substrate consisting essentially of, by weight percent, from about 0.01 percent to about 0.13 percent carbon, from about 0.5 percent to about 3 percent chromium, from about 0.8 percent to about 3 percent aluminum, from about 0.4 percent to about 1.5 percent silicon, from about 0.1 percent to about 0.6 percent manganese, from about 0.1 percent to about 0.5 percent titanium, and remainder iron except for incidental impurities.

2. An article in sheet form having good oxidation resistance at elevated temperature, good resistance against attack by hydrocarbon combustion products at elevated temperature, good formability, good weldability, and high strength, said article consisting of an outer layer applied by hot dip coating chosen from the class consisting of aluminum, and aluminum alloys, and a ferritic substrate consisting essentially of, by weight percent, from about 0.04 percent to about 0.06 percent carbon, from about 1.7 percent to about 2.1 percent chromium, from about 1.7 percent to about 2.0 percent aluminum, from about 0.6 percent to about 0.9 percent silicon, from about 0.2 percent to about 0.4 percent manganese, from about 0.1 percent to about 0.6 percent titanium, with the titanium content being about 8 times the carbon content, and remainder iron, except for incidental impurities.

3. Articles for high temperature applications such as space heaters, automotive exhaust systems, and the like, said articles comprising an outer hot dip coating chosen from the class consisting of aluminum, and aluminum alloys, the weight of said coating being about  $\frac{1}{2}$  ounce per square foot of sheet, and a cold reduced and annealed ferritic sheet metal base consisting essentially of, by weight percent, from about 0.01 percent to about 0.13 percent carbon, from about 0.5 percent to about 3 percent chromium, from about 0.8 percent to about 3 percent aluminum, from about 0.4 percent to about 1.5 percent silicon, from about 0.1 percent to about 0.6 percent manganese, from about 0.1 percent to about 1 percent titanium, and remainder iron except for incidental impurities.

4. The articles claimed in claim 3, wherein said sheet metal base consists essentially of, by weight percent, from about 0.04 percent to about 0.06 percent carbon, from about 1.7 percent to about 2.1 percent chromium, from about 1.7 percent to about 2.0 percent aluminum, from about 0.6 percent to about 0.9 percent silicon, from about 0.2 percent to about 0.4 percent manga-

nese, from about 0.1 percent to about 0.6 percent titanium, with the titanium content being about 8 times the carbon content, and remainder iron except for incidental impurities, said articles having good oxidation resistance at elevated temperature, good formability, good weldability, good resistance against attack by hydrocarbon combustion products at elevated temperature, and high strength.

5. The articles claimed in claim 3, wherein an element chosen from the class consisting of columbium, zirconium, and mixtures thereof is substituted at least partially for titanium in a stoichiometrically equivalent amount.

\* \* \* \* \*

10

15

20

25

30

35

40

45

50

55

60

65